

[54] **PROCESS FOR THE MANUFACTURE OF ALUMINIUM ELECTRODES FOR ELECTROLYTIC CAPACITORS**[75] Inventors: **Martin Mühlhäuser, Singen, Hohentw; Christian Roth, Gottmadingen, both of Germany**[73] Assignee: **Aluminium-Walzwerke Singen GmbH, Singen/Hohentw, Germany**[22] Filed: **Nov. 7, 1973**[21] Appl. No.: **413,447**[30] **Foreign Application Priority Data**

Nov. 11, 1972 Germany ..... 2255309

[52] U.S. Cl. ..... **204/129.75; 29/527.7; 29/570; 29/DIG. 10**[51] Int. Cl. .... **C01b 13/04**[58] **Field of Search ... 29/527.7, 570, 592, DIG. 16; 164/82; 204/129.75**

[56]

**References Cited****UNITED STATES PATENTS**

|           |         |                    |              |
|-----------|---------|--------------------|--------------|
| 1,935,860 | 11/1933 | Robinson .....     | 29/570       |
| 2,106,178 | 1/1938  | Keller et al. .... | 29/570 X     |
| 2,206,050 | 7/1940  | Robinson .....     | 29/570       |
| 3,316,164 | 4/1967  | Welch .....        | 204/129.75 X |
| 3,351,442 | 11/1967 | Hooper .....       | 204/129.75 X |

*Primary Examiner*—Milton S. Mehr*Assistant Examiner*—D. C. Reiley, III*Attorney, Agent, or Firm*—Ernest F. Marmorek

[57]

**ABSTRACT**

A process for the manufacture of etched aluminium electrodes for electrolytic capacitors wherein the strips to be etched are cast directly as a strip from the molten state and then rolled to the final thickness before electrolytically etching them in the presence of chloride ions.

**1 Claim, No Drawings**

**PROCESS FOR THE MANUFACTURE OF  
ALUMINIUM ELECTRODES FOR ELECTROLYTIC  
CAPACITORS**

The electrodes of an electrolytic capacitor generally consist of a roughened i.e. etched aluminium strip. By roughening the strip an increase in surface area and thereby an increase in capacity is achieved, or for a prescribed capacity a reduction in the dimension of the electrode is achieved.

Pure aluminium is normally used as starting material for producing etched anode strips and for the production of etched cathode strip pure aluminium or manganese-containing aluminium alloys are used. These materials are cast as ingots with rectangular cross section by the usual continuous casting and permanent mould casting processes. The ingots are usually heated to a rolling temperature between 400°C and 500°C and rolled down to a plate thickness of 2-10 mm on a hot rolling mill. The plates are cold rolled in several reduction passes down to strip thickness and etched either in this condition or after an additional heat treatment.

The etched strips produced in this way do not, in many cases fulfill today's requirements for a satisfactory surface area increase necessary in the construction of an electrolytic capacitor of the smallest possible volume. It was of value therefore to find a process by which it is possible to obtain still greater increases in the surface area than by the known processes.

surface area. It is characterised in that the aluminium strip to be etched is cast directly from the molten state as a strip and then rolled to its final thickness.

Presumably the better etching behaviour of the material produced by strip-casting results from the significantly higher rate of solidification during casting.

**EXAMPLES**

An ingot of 99% pure aluminium and an ingot of 10 AlMn alloy, both continuously cast, were annealed at 500°C for 2 hours, hot rolled to a plate thickness of 6 mm and then without heat treatment cold rolled to a strip 0.05 mm thick. For comparison a strip from a melt of 99% pure aluminium and a strip from an AlMn 15 melt were cast directly as 7 mm thick strips in a strip-casting plant and then rolled down to the same final thickness as the other two strips without an intermediate heat treatment. All strips were degreased and then etched in an aqueous solution of 20% NaCl at 90°C 20 using a current density of 100 A/dm<sup>2</sup> and consuming 3000 C/dm<sup>2</sup>.

The determination of the capacity was carried out in accordance with the DIN 41330 specification at 0 and 10 volts in a saturated ammonium pentaborate solution 25 having a bath resistance of 60 to 70 ohm.cm at room temperature. In addition to this the characteristic data for the mechanical properties of the strips were determined before etching. The results are summarized in the following tables.

Example 1 (Al 99)

|               | $\sigma B$<br>(kp/mm <sup>2</sup> ) | $\delta 100$<br>(%) | Capacity in $\mu F/cm^2$                          |                |
|---------------|-------------------------------------|---------------------|---------------------------------------------------|----------------|
|               |                                     |                     | in accordance with the DIN<br>41330 specification | 0 Volt 10 Volt |
| Ingot casting | 23,2                                | 3,3                 |                                                   |                |
| Strip casting | 24,0                                | 3,4                 | 150                                               | 40             |

Example 2 (AlMn)

|               | $\sigma B$<br>(kp/mm <sup>2</sup> ) | $\delta 100$<br>(%) | Capacity in $\mu F/cm^2$                          |                |
|---------------|-------------------------------------|---------------------|---------------------------------------------------|----------------|
|               |                                     |                     | in accordance with the DIN<br>41330 specification | 0 Volt 10 Volt |
| Ingot casting | 32,5                                | 2,5                 |                                                   |                |
| Strip casting | 32,9                                | 3,8                 | 350                                               | 100            |

For some years in addition to the above mentioned casting of ingots, a continuous casting of strip has been practised. By this latter technique a material is cast directly from the melt in the form of a strip 1-40 mm 55 thick and then hot rolled and cold rolled or directly cold rolled to its final thickness.

It was found on comparison of the aluminium strip made from cast strips with those made from cast ingots that the former showed a significantly greater increase in the surface area after the same etching treatment. This effect is to be found not only with pure aluminium but also with aluminium alloys.

The instant invention concerns therefore a process for the production of aluminium electrodes for electrolytic capacitors utilizing a process wherein the electrodes are etched electrolytically in a chloride-containing electrolyte for the purpose of increasing the

The results show that the mechanical strength after solidifying is independent of the method of casting. The result of etching and the capacity measurement on the other hand show clearly an increase in capacity in the case of the metal strip produced by the strip-casting process.

What is claimed is:

1. A process for the manufacture of aluminum electrodes, for use in electrolytic capacitors, comprising the steps of

continuously casting an aluminum strip having a thickness of between about 1 mm and about 40 mm; rolling said aluminum strip to its final thickness; and etching said rolled strip electrolytically in a chloride containing electrolyte.

\* \* \* \* \*